

# UNITED STATES PATENT OFFICE.

ROBERT DEMUTH, OF NEW YORK, N. Y., ASSIGNOR TO THE FARBNFABRIKEN, VORMALS FR. BAYER & CO., OF SAME PLACE.

## BROWN SULFUR DYE.

SPECIFICATION forming part of Letters Patent No. 603,755, dated May 10, 1898.

Application filed October 16, 1896. Serial No. 609,162. (Specimens.) Patented in Italy January 13, 1896, XXXI, 40,624, LXXIX, 407, and in France January 15, 1896, No. 253,213.

*To all whom it may concern:*

Be it known that I, ROBERT DEMUTH, chemist, doctor of philosophy, a subject of the Emperor of Germany, (assignor to the FARBNFABRIKEN, VORMALS FR. BAYER & CO., of Elberfeld, Prussia, Germany,) temporarily residing in the city, county, and State of New York, have invented a new and useful Improvement in the Manufacture of Brown Coloring-Matters, (for which the aforesaid Farbenfabriken, vormalis Fr. Bayer & Co., have already obtained Letters Patent in France, No. 253,213, dated January 15, 1896, and in Italy, Reg. Gen., Vol. XXXI, No. 40,624, Reg. Att., Vol. LXXIX, No. 407, dated January 13, 1896;) and I do hereby declare the following to be an exact and clear description of my invention.

My invention relates to the production of new brown coloring-matter dyeing cotton at ordinary temperature and resulting by the action of either sulfur and alkalies or alkaline sulfids or mixtures of sulfur and alkaline sulfids on cresol.

In the manufacture of the new dye I use the crude cresol or ortho cresol, meta cresol, para cresol, or any mixture whatever thereof. Naturally the crude cresol will be mostly used for cheapness sake. The dyes thus obtained have nearly the same properties and are of considerable technical value, as they are capable of dyeing vegetable fiber or fabrics at ordinary temperature and do not require any handling of the goods to be dyed. They yield on vegetable fiber or fabric in cold dyeing-baths, with or without an addition of alkaline sulfid, brown shades distinguished by their intensity and fastness.

In carrying out this invention I can proceed, for instance, as follows: Ten parts (the parts are by weight) of crude cresol are mixed with twenty-five parts of sulfur and fifty parts of a solution of soda, (containing about sixty per cent. of NaOH.) The resulting mixture is gradually heated, preferably in a fusion vessel provided with a reflux condenser, to about 270° centigrade. This gradual heating is necessary, because at certain temperatures a violent action of the liquid ensues. Upon the subsidence of this action the temperature is again raised. The process is continued until

the desired temperature is reached. If after, say, four hours the melt has assumed the aforesaid temperature—viz., 270° centigrade—the mass is kept at this temperature for about two hours. The resulting melt forms a solid mass, which, after cooling and pounding to pieces, can be used directly for dyeing purposes. The dyestuff thus obtained in the form of its sodium salt forms a black mass readily soluble in water, affording a greenish-black or bluish-black colored solution. The said solution dyes cotton a brown at ordinary temperature, and these shades are fast against washing. Moreover, it is not necessary to handle the goods to be dyed while being in the dyeing-bath, as the color strikes evenly on the fiber if the material is placed in the dyeing-bath and kept therein for several hours.

On acidulating the aqueous solution of the dyestuff with mineral acids—for instance, muriatic acid—the dyestuff in the so-called “free state” is separated as a black precipitate, which when dried forms a brownish-black powder. This powder is insoluble in water, sodium carbonate, ammonia, and alcohol. It dissolves with difficulty in dilute soda-lye at ordinary temperature, more easily in hot soda-lye, producing a greenish-brown-colored liquid. It is dissolved with readiness by solutions of alkaline sulfids—for instance, sodium sulfid—a greenish-brown-colored liquid being thus obtained. In concentrated sulfuric acid at 66° Baumé it is insoluble or soluble with difficulty. Its solutions in alkaline sulfids possess the same dyeing properties as the aqueous solutions of the melt obtained as hereinbefore described—that is to say, they dye cotton at ordinary temperature a fast brown.

Although in the above example I have described crude cresol as the product to start from, (which will be mostly the case in practically manufacturing this dye,) ortho cresol, meta cresol, para cresol, or any mixture whatever thereof can be used. The resulting products possess almost the same properties and also yield on cotton at ordinary temperature fast brown shades. The mode of working, the quantities of the materials used, and the

temperature above referred to can vary within certain limits. The process proceeds in an analogous manner if potassa is used in place of soda or if alkaline sulfids or mixtures of 5 sulfur and alkaline sulfids are allowed to act on cresol.

Having fully described my invention, what I claim, and desire to secure by Letters Patent, is—

- 10 1. The process of producing a new coloring-matter in the form of alkaline salts capable of dyeing vegetable fiber or fabrics at ordinary temperatures fast brown shades, which process consists in subjecting cresols and sulfur in 15 strong alkaline liquid to temperatures above 200° centigrade, substantially as described.
2. As a new article of manufacture the brown coloring-matter producible from cresols and sulfur in alkaline solution at temperatures above 200° centigrade, being in the 20 form of its alkaline salts a black mass easily soluble in water with a greenish-black or

bluish-black color capable of dyeing cotton fabrics at ordinary temperatures fast brown shades, and having when precipitated with acids, the characteristics of a brownish-black powder insoluble in water, sodium carbonate, ammonia, and alcohol, soluble with difficulty in dilute soda-lye at ordinary temperature, more easily soluble in hot soda-lye with 25 a greenish-brown color, insoluble or soluble with difficulty in concentrated sulfuric acid (66° Baumé), easily soluble with a greenish-brown color in alkaline sulfids, thus affording solutions which dye cotton at ordinary 30 temperatures in fast brown shades substantially as described.

In testimony whereof I have signed my name to this specification in the presence of two subscribing witnesses.

ROBERT DEMUTH.

Witnesses:

ERNEST HOPKINSON,  
W. LAIRD GOLDSBOROUGH.